



US010793961B2

(12) **United States Patent**  
**Froelicher et al.**

(10) **Patent No.:** **US 10,793,961 B2**  
(45) **Date of Patent:** **Oct. 6, 2020**

(54) **METHOD OF OBTAINING A 18 CARATS 3N GOLD ALLOY**

(71) Applicant: **The Swatch Group Research and Development Ltd**, Marin (CH)

(72) Inventors: **Thomas Froelicher**, Le Landeron (CH); **Christophe Henzirohs**, Sonceboz (CH); **Guido Plankert**, Boppelsen (CH)

(73) Assignee: **The Swatch Group Research and Development Ltd**, Marin (CH)

(\*) Notice: Subject to any disclaimer, the term of this patent is extended or adjusted under 35 U.S.C. 154(b) by 169 days.

(21) Appl. No.: **16/038,662**

(22) Filed: **Jul. 18, 2018**

(65) **Prior Publication Data**

US 2018/0320283 A1 Nov. 8, 2018

**Related U.S. Application Data**

(62) Division of application No. 13/427,558, filed on Mar. 22, 2012, now Pat. No. 10,053,789.

(30) **Foreign Application Priority Data**

Mar. 31, 2011 (EP) ..... 11160669

(51) **Int. Cl.**

**B32B 15/01** (2006.01)

**C25D 3/62** (2006.01)

(52) **U.S. Cl.**

CPC ..... **C25D 3/62** (2013.01)

(58) **Field of Classification Search**

USPC ..... 420/511

See application file for complete search history.

(56) **References Cited**

**U.S. PATENT DOCUMENTS**

|                 |   |         |                  |       |           |
|-----------------|---|---------|------------------|-------|-----------|
| 2,127,676 A     | * | 8/1938  | Coleman          | ..... | C22C 5/02 |
|                 |   |         |                  |       | 148/577   |
| 3,642,589 A     |   | 2/1972  | Nobel et al.     |       |           |
| 4,980,035 A     |   | 12/1990 | Emmenegger       |       |           |
| 5,045,411 A     | * | 9/1991  | Taylor           | ..... | C22C 5/02 |
|                 |   |         |                  |       | 420/481   |
| 5,256,275 A     | * | 10/1993 | Brasch           | ..... | C25D 3/62 |
|                 |   |         |                  |       | 205/247   |
| 2005/0184369 A1 |   | 8/2005  | Sonoda et al.    |       |           |
| 2006/0283714 A1 |   | 12/2006 | Egli et al.      |       |           |
| 2012/0247968 A1 |   | 10/2012 | Foelicher et al. |       |           |

**FOREIGN PATENT DOCUMENTS**

|    |              |         |
|----|--------------|---------|
| EP | 0 416 342 A1 | 3/1991  |
| EP | 0 566 054 A1 | 10/1993 |
| EP | 1 728 898 A2 | 12/2006 |
| EP | 2 312 021 A1 | 4/2011  |
| JP | 62-164890 A  | 7/1987  |
| JP | 09310166 A   | *       |
|    |              | 12/1997 |

**OTHER PUBLICATIONS**

European Search Report of EP 11 16 0669, dated May 26, 2011.

\* cited by examiner

*Primary Examiner* — Seth Dumbris

(74) *Attorney, Agent, or Firm* — Sughrue Mion, PLLC

(57) **ABSTRACT**

A method for the galvanoplastic deposition of a gold alloy on an electrode dipped into a bath including gold metal, organometallic compounds, a wetting agent, a sequestering agent and free cyanide, the alloy metals being copper metal and silver metal allowing a mirror-bright yellow gold alloy to be deposited on the electrode characterized in that the bath respects a proportion of 21.53% gold, 78.31% copper and 0.16% silver.

**9 Claims, No Drawings**

## 1

## METHOD OF OBTAINING A 18 CARATS 3N GOLD ALLOY

## CROSS REFERENCE TO RELATED APPLICATIONS

This is a divisional of application Ser. No. 13/427,558, filed Mar. 22, 2012, which claims priority from European Patent Application No. 11160669.5 filed Mar. 31, 2011, the entire disclosures of which are incorporated herein by reference.

## FIELD OF THE INVENTION

The invention relates to electrolytic deposition in the form of a thick gold alloy layer and the method of fabricating the same.

## BACKGROUND OF THE INVENTION

In the field of decorative plating, methods are known for producing yellow coloured, electrolytic depositions of gold, with a grade equal to or more than 9 carats, which is ductile, with a thickness of 10 microns and with a high level of tarnish resistance. These depositions are obtained by electrolysis in an alkaline galvanic bath containing 0.1 to 3 g·l<sup>-1</sup> cadmium, in addition to gold and copper.

The depositions obtained by these known methods have, however, a cadmium content of between 1 and 10%. Cadmium facilitates deposition of thick layers, i.e. between 1 and 800 microns and provides a yellow coloured alloy while reducing the quantity of copper contained in the alloy. However, cadmium is extremely toxic and prohibited in some countries.

18 carats gold alloys without any cadmium, which contain copper and zinc, are also known. However, these depositions have an excessively pink hue (too rich in copper). Finally, these depositions have poor corrosion resistance which means they tarnish quickly.

## SUMMARY OF THE INVENTION

It is an object of the present invention to overcome all or part of the aforementioned drawbacks, by providing a manufacturing method for depositing a thick, 3N yellow coloured, 18 carats gold alloy layer which has neither zinc nor cadmium as its main constituents.

The invention therefore relates to a method for the galvanoplastic deposition of a gold alloy on an electrode dipped into a bath including gold metal, organometallic compounds, a wetting agent, a sequestering agent and free cyanide, the alloy metals being copper metal and silver metal allowing a mirror-bright yellow gold alloy to be deposited on the electrode characterized in that the bath respects a proportion of 21.53% gold, 78.31% copper and 0.16% silver.

Thus, surprisingly, the bath even based on high copper concentration is able, advantageously according to the invention, to achieve a 3N yellow gold alloy in respecting a proportion of 21.53% gold, 78.31% copper and 0.16% silver and a 5N red gold alloy.

According to other advantageous features of the invention:

the bath includes from 1 to 10 g·l<sup>-1</sup> of gold metal in double gold and potassium cyanide form;

the bath includes from 10 to 60 g·l<sup>-1</sup> of copper metal in copper iodide form;

## 2

the bath includes from 10 mg·l<sup>-1</sup> to 1 g·l<sup>-1</sup> of silver metal in double silver and potassium cyanide form;

the bath includes from 3 to 35 g·l<sup>-1</sup> of cyanide;

the wetting agent has a concentration of between 0.05 and 10 ml·l<sup>-1</sup>

the wetting agent is chosen from among polyoxyalkenic, ether phosphate, lauryl sulphate, dimethyldodecylamine-N-oxide, dimethyl(dodecyl) ammonium propane sulfonate;

the bath includes a concentration of amine of between 0.01 and 5 ml·l<sup>-1</sup>;

the bath includes a concentration of depolariser of between 0.1 and 20 mg·l<sup>-1</sup>;

the bath includes phosphate, carbonate, citrate, sulphate, tartrate, gluconate and/or phosphonate type conductive salts;

the temperature of the bath is kept between 50 and 90° C.; the pH of the bath is kept between 8 and 12;

the method is performed at a current density of between 0.05 to 1.5 A·dm<sup>-2</sup>;

The invention also concerns an electrolytic deposition in the form of a gold alloy obtained from a method according to any of the preceding claims, the thickness of which is between 1 and 800 microns and which includes copper, characterized in that it includes silver as the third main compound and in that the deposition is made of 75% gold, 19% copper and 6% silver, allowing a bright 3N colour to be obtained.

## DETAILED DESCRIPTION OF THE PREFERRED EMBODIMENTS

The invention concerns an electrolytic deposition of a gold alloy with a 3N colour which, surprisingly, includes Au—Cu—Ag as its respective main compounds in proportions that are not known, to obtain the 3N colour, i.e. bright yellow.

In the example deposition above, there is a gold alloy, free of toxic metals or metalloids, and in particular free of cadmium and zinc, with a 3N yellow colour, a thickness of 200 microns, excellent brightness and with a very high level of resistance to wear and tarnishing.

This deposition is obtained by electrolysis in an electrolytic bath of the type:

Au: 5.5 g·l<sup>-1</sup>;

Cu: 20 g·l<sup>-1</sup>;

Ag: 40 mg·l<sup>-1</sup>;

CN: 5 g·l<sup>-1</sup>;

pH: 10.5;

Temperature: 80° C.;

Current density: 0.3 A·dm<sup>-2</sup>;

Wetting agent: 0.05 ml·l<sup>-1</sup> NN-Dimethyldodecyl N-oxide;

Iminodiacetic: 20 g·l<sup>-1</sup>;

Ethylenediamene: 0.5 ml·l<sup>-1</sup>;

Gallium, selenium or tellurium: 10 mg·l<sup>-1</sup>.

Consequently, the bath respects a proportion of 21.53% gold, 78.31% copper and 0.16% silver between its main compounds.

The electrolysis is preferably followed by a heat treatment at a temperature of between 200 and 450 degrees Celsius for 1 to 30 minutes in order to obtain a deposition of optimum quality.

These conditions provide a cathodic yield of 95 mg·A·min<sup>-1</sup> with a deposition speed of around 10 µm per hour in the case of the example.

Thus, surprisingly, the bath according to the invention provides a deposition in proportions of around 75% gold,

19% copper and 6% silver, corresponding to a 3N colour, 18 carat deposition, very different proportions from the usual electrolytic depositions for this colour, which tend to be depositions of around 75% gold, 12.5% copper and 12.5% silver.

The bath may also contain a brightener. This is preferably a butynediol derivative, a pyridinio-propanesulfonate or a mixture of the two, a tin salt, sulfonated castor oil, methylimidazole, dithiocarboxylic acid such as thiocarbamide, thiobarbituric acid, imidazolidinethione or thiomalic acid.

In these examples, the electrolytic bath is contained in a polypropylene or PVC bath holder with a heat insulating coating. The bath is heated using quartz, PTFE, porcelain or stabilised stainless steel thermo-plungers. Good cathodic rod movement and electrolyte flow must be maintained. The anodes are made of platinum plated titanium, stainless steel, ruthenium, iridium or alloys of the latter two.

Of course, the present invention is not limited to the illustrated example but is capable of various variants and alterations which will be clear to those skilled in the art. In particular, the bath may contain the following metals: Zr, Se, Te, Sb, Sn, Ga, As, Sr, Be, Bi in negligible quantities.

Moreover, the wetting agent may be of any type that can wet in an alkaline cyanide medium.

What is claimed is:

1. A gold alloy, the gold alloy being a bright 3N yellow gold alloy composition of 75% gold, 19% copper and 6% silver.

2. The gold alloy according to claim 1, wherein the gold alloy has thickness of from 1 to 800 microns.

3. An electrolytic deposition comprising: a galvanoplastically deposited gold alloy layer on an electrode, the gold alloy being a bright 3N yellow gold alloy composition of 75% gold, 19% copper and 6% silver.

5. The electrolytic deposition according to claim 3, wherein the gold alloy layer has a thickness of from 1 to 800 microns.

10 6. An electrolytic deposition comprising: a galvanoplastically deposited gold alloy layer on an electrode, wherein the gold alloy is a bright 3N yellow gold alloy composition of 75% gold, 19% copper and 6% silver, and a structure of the gold alloy composition is obtained by a method comprising:

- (a) providing the electrode;
- (b) dipping the electrode into a bath, wherein the bath includes gold metal, copper metal, silver metal, organometallic compounds, a wetting agent, a sequestering agent and free cyanide; and
- (c) galvanoplastically depositing the gold alloy layer on the electrode.

15 20 7. The electrolytic deposition according to claim 5, wherein the gold alloy layer has a thickness of from 1 to 800 microns.

8. The gold alloy according to claim 1, wherein the gold alloy composition is free of cadmium and free of zinc.

9. The electrolytic deposition according to claim 5, wherein the gold alloy composition is free of cadmium and free of zinc.

\* \* \* \* \*